

April 28, 1942.

H. S. COOPER

2,281,235

PROCESS OF FUSING OF BERYLLIUM CHLORIDE

Filed Nov. 28, 1940



INVENTOR  
HUGH S. COOPER

BY  
*Bair, Borden & Fox*  
ATTORNEY

## UNITED STATES PATENT OFFICE

2,281,235

## PROCESS OF FUSING BERYLLIUM CHLORIDE

Hugh S. Cooper, New York, N. Y., assignor to  
 Cooper-Wilford Beryllium, Ltd., Philadelphia,  
 Pa., a corporation of Delaware

Application November 28, 1940, Serial No. 367,623

1 Claim. (Cl. 263—52)

This invention relates to the production of fused beryllium chloride.

An object of this invention is to make a form of anhydrous beryllium chloride that is less reactive with the atmosphere than has been possible with the formation of beryllium chloride according to the prior art.

Another object is to effect a fused form of beryllium chloride.

Still another object is to produce a form of beryllium chloride particularly effective for easy and economical production of beryllium therefrom.

Other objects and advantages will be apparent from the following specification.

The drawing represents an illustrative diagrammatic section of the apparatus with which the method of this invention is practised.

In the manufacture of pure beryllium metal the common method is the electrolysis of anhydrous beryllium chloride in a suitable fused salt bath. For this and other purposes the anhydrous chloride is made by the chlorination of the oxide or other oxy-compound of beryllium, usually at a temperature between 800° C. and 1000° C. Since the vaporization temperature of the chloride is far below its temperature of formation in the chlorinator, it is of necessity recovered by condensation. This produces a light, fluffy, and highly porous mass of thin needle crystals. In this form the chloride is extremely reactive with the atmosphere and can be stored for only a short time without deterioration, and only then by the exercise of extreme precautions and care. The use of this chloride of the prior art in an electrolytic bath for the making of beryllium is also a matter of considerable difficulty. When it is added to the bath it tends to float on the surface where it vaporizes and oxidizes instead of going quickly into solution. The part that does go into solution gives up its entrained moisture causing the bath to froth and sometimes run over the sides of the container.

These and other difficulties of the storage and use of beryllium chloride are overcome by its use in massive fused form. Since beryllium chloride vaporizes directly from the solid however, and its liquid phase and is not easily obtainable under ordinary conditions, the melting of it is not normally either a simple or an easy procedure, but it is rendered both simple and easy by means of the present invention.

In the practice of this invention a metal cylinder is used such as is shown in the cross sectional view attached. This cylinder can con-

veniently be made of steel. The cylinder 1 is permanently closed at the bottom end. At its top the cylinder has a removable cap 2 held tightly in place by any convenient means, as for instance, the bolts 3 and the flange 4. Drilled through the cap 2 is a hole 5 into which is screwed a short piece of pipe 6. At its other end the pipe 6 carries a valve 7, which in turn communicates with a short piece of pipe 8, used to carry away effluent gases. If desired the valve 7 may be an automatic check valve preventing gases from travelling inward toward the cylinder.

Inside the cylinder 1 is a liner 9 which can conveniently be made of sheet iron or the like. 15 This liner also comprises a cylinder closed at the bottom only. This liner fits loosely into the cylinder 1 with its bottom resting on the bottom of the cylinder. The liner 9 is filled with the ordinary fluffy beryllium chloride 10, in the form 20 in which it comes from the chlorinator. This chloride is tamped in place to increase the content as much as is conveniently possible.

After the liner has been filled and placed in the cylinder, the cap 2 is securely fastened in place. The whole assembly is then placed in any suitable furnace such as is described below and is so arranged that the cap 2 and its attached valve 7 and pipes 6 and 8 all protrude outside the furnace while the balance of the cylinder and its 30 contained liner filled with beryllium chloride are inside the furnace. A suitable furnace is shown in the drawing in which 11 is the furnace shell, preferably made of steel, having a refractory lining 12 and provided with a refractory cover 13 with a hole arranged to receive the steel cylinder. The furnace is fired as by a suitable burner 14 say, for gas or oil having flame projection 15 as will be clear.

Heat is now applied to the furnace and at the 40 same time the valve 7 is opened just a crack. After a little while when the interior of the cylinder has reached a temperature of about 100° C., fumes will start to be emitted from the chloride which will issue from the pipe 8. These 45 vapors or gases consist largely of steam and a little hydrogen chloride vapor, and are allowed to escape. As the temperature in the cylinder approaches 300° to 400° C., the fumes become more dense. They now consist largely of vaporized beryllium chloride and the change in the character of the fumes indicates that the contained moisture has largely been driven off. At this 50 point the valve 7 may be closed tightly without risk of building up any dangerous pressure in the cylinder. The heating is continued for a time

longer, to make sure that all parts of the cylinder have reached a temperature of about 400° C., but without greatly exceeding that temperature. The valve 7 is tightly closed before the furnace is opened, in any case, and certainly before any drop in temperature is permitted internally of the cylinder 4.

The cylinder is now removed from the furnace and permitted to cool. The cap 2 is then removed and the liner 3, with its contents, is withdrawn from the cylinder. In the bottom of the liner is found a solid fused mass of beryllium chloride. It adheres very tightly to the sheet iron of the liner but it can be removed by hammering the sides of the liner. The material so recovered is completely solid, and relatively hard and dense.

In the atmosphere it deteriorates only very slowly, particularly if it is kept in the form of lumps. When it is added to a fused electrolytic bath it dissolves very rapidly with negligible vaporization, frothing, or oxidation, and results in larger electrolytic yields of metal.

Having described my invention the claim is as follows:

10 The process of fusing beryllium chloride which comprises heating it in a closed vessel to a temperature of about 300° C. while permitting the generated vapors to escape, and thereafter heating to a temperature of about 400° C. while keeping the vessel tightly closed.

HUGH S. COOPER.